# EUROPEAN PATENT SPECIFICATION

(11) **EP 0 259 069 B1**
(45) Date of publication and mention of the grant of the patent: **09.12.1992**
(21) Application number: 87307378.7
(22) Date of filing: 20.08.1987
(51) Int. Cl.: B27N 3/04

(54) **Waferboard lumber**
Holzfaserbauholz
Bois de charpente de fibres de bois

(30) Priority: 03.09.1986 CA 517415
(43) Date of publication of application: 09.03.1988
(73) Proprietor: MACMILLAN BLOEDEL LIMITED, Vancouver British Columbia V6E 3R9 (CA)
(72) Inventor: Barnes, Derek, Vancouver B.C. V6P 2A7 (CA)
(74) Representative: Heath, Derek James

(56) References cited:
- DE-A- 3 323 639
- FR-A- 1 011 675
- US-A- 4 122 236
- US-A- 4 241 133
- US-A- 4 255 477
- US-A- 4 492 726
- US-A- 4 494 919
- US-A- 4 610 913
- US-A- 4 751 131
- PATENT ABSTRACTS OF JAPAN, vol. 5, no. 39 (M-59)[711], 14th March 1981; & JP-A-55 164 141 (MASAO TAKAHASHI) 20-12-1980
- Thomas M. MALONEY "Modern Particleboard & Dry-process Fiberboard Manufacturing", 1977, MILLER FREEMAN PUBLICATIONS, pages 178-216

## Description

The present invention relates to waferboard lumber, more particularly the present invention relates to lumber products formed from wafers oriented to be substantially parallel to the longitudinal axis of the lumber product and a method of producing such product.

### BACKGROUND TO THE PRESENT INVENTION

There have been many patents issued and many papers published on the manufacture of lumber-like products from wood particles. Similarly it is common practice to manufacture waferboard-type panel products from wood particles and there have been a number of articles published.

In the realm of oriented strandboard, the normal practice has been to manufacture a board from particles having a maximum length of up to about 4 inches (100 mm) and many papers and articles have been published advocating 4 inches (100 mm) as a maximum length of wafer. However, in a recently filed United States Patent application 829,564 which is a continuation of application number 723,641 filed April 16, 1985, applicant has taught major advantages can be obtained utilizing long wafers in forming a layered waferboard product.

Australian patent 136,844 issued March 28, 1950 is one of the earlier disclosures relating to the manufacture of lumber from particles. In this patent the particles recommended are sticks, twigs, etc that are oriented in the longitudinal direction of the lumber and secured together. It has also been proposed in Czechoslovakian patent number 93,154 issued December 15, 1959 to Stofko, to produce a moulded product by orienting wood elements in what are broadly defined as profiles such as I, U, T, L and others including pipes and windows, and pressing to consolidate into a finished or semifinished product. The teachings of this patent are further amplified by articles published by Stofko in Drevarsky Dyskum 2 No. 1:81-102 (1957); Drevarsky Dyskum 5 No 2:241-261 (1960)., Drevarsky Dyskum 2:127-148 (1962) and Drvna Industriaja 21 (6):104-107 (1970). In these articles Stofko discusses panel products and lumber products presumably moulded as taught in his patent and emphasizes the importance of slenderness ratio, i.e. the ratio of length to thickness of the wood particles to obtain the desired structural properties at an acceptable density.

United States patent 3,164,511 issued January 7, 1965 to Elmendorf discloses the manufacture of a lumber product from wafers having length of up to about 6 inches (150 mm), width up to about 1/4 inch (150 mm) and thicknesses between 0.005 to 0.02 inches (0.1 to 0.5 mm). To applicant's knowledge no commercial lumber products utilizing such wood particles have been manufactured and sold.

U.S. patent 3,956,555 issued May 11, 1976 to McKeen describes the manufacture of a laminted beam from a combination of oriented and random wood particles in a press by laying alternative strips of oriented and random particles and then consolidating under pressure to form a panel and splitting the oriented strips to divide the panel in to structures having end side sections that are oriented and would function similar to flanges of an I beam interconnected by a random oriented section that would function as the web of an I beam. This is a relatively complicated structure with limited strength and suitable only for use with the products oriented to be loaded perpendicular to the split faces.

As far as applicant is aware, the product described in U.S. patent 4,061,819 issued December 6, 1977 to the present inventor describes the only commercially viable suitable lumber product formed from wood particles (strands). This patent teaches the use of relatively long strands to obtain structural products having physical characteristics including density and strength characteristics similar to, and in some cases better than, those of the natural wood product it replaces.

United States patent 4,122,236 issued October 24, 1978 to Holman describes an artificial lumber product moulded from splinters having a length in the range of about 2 to 10 inches.

Generally when waferboards (panels) or the like are made, the density profile through the panel is such that the skins of the panel have maximum density and the core has the least density. Stated another way, the strength of the skins of the panel is higher than the strength of core, however, since panels are normally used with the core extending along the neutral axis of the bending moment such a density distribution is not a major factor in determining bending strength. It is known that the rate of pressure application in a press can be used to change the density profile through the thickness of the panel. Also in a continuous pressing operation the rate of temperature rise coordinated with the rate of pressure application can be used to change the density profile with thickness to the panel.

It is economical to produce wafers since the wafers are normally produced by a blade having spaced edges equal in length to the length of the wafer to be produced cutting substantially parallel to the grain. In some cases flat blades cutting parallel to the grain are used with spaced spurs cutting perpendicular to the grain to define the length of the wafers. Wafers so produced are generally relatively thin and have a width many times greater than their thickness (thickness being determined by the depth of cut of the blade and the width being determined by the deflection of the cut wafer by the breaker bar of the knife).

### BRIEF DESCRIPTION OF THE PRESENT INVENTION

It is an object of the present invention to provide a lumber product formed utilizing waferboard technology and wafers having the following average geometry; length at least 8 inches (200 mm) maximum thickness of 0.15 inches (4 mm) and a width of at least 0.25 inches (6 mm) to provide a relatively inexpensive lumber product having physical characteristics similar to or better than those obtained from lumber made from the same species as the wood flakes.

Broadly the present invention relates to a waferboard lumber product and a method of making same, said waferboard lumber product comprising discrete lengths of lumber having thicknesses of at least 1 inch (25 mm) made from a single layer panel formed from wood wafers, said wafers being oriented to have their lengths orientated to the longitudinal length of the panel measured in the major plane of said panel with a mean deviation of 0 to 10 degrees and a mean deviation measured in a minor longitudinal plane through the panel perpendicular to the said major plane of from 0 to 5 degrees, said wafers having an average effective length of at least 8 inches (200 mm) said lengths of lumber having cut edges defined in said panel by cuts extending substantially longitudinally of said panel said cuts being spaced defined the width of said lumber.

Preferably said wafers will have a maximum average thickness of 0.15 inches (4 mm) and an average width of at least 0.25 inches (6 mm).

Preferably said lumber product will have a substantially uniform density to thickness profile.

Present invention also relates to a method of making a lumber product comprising laying up a single layer panel having a thickness of at least 1 inch (25 mm) from a plurality of wafers, orienting the longitudinal length of said wafers relative to the longitudinal axis of said panel so that the mean deviation of the lengths of said wafers to said longitudinal axis of said panel measured in the major plane of said panel is in the range of 0 to 10 degrees and a mean deviation measured in a longitudinal plane through said panel perpendicular to said major plane of from 0 to 5 degrees, said wafers having an average effective length of at least 8 inches (200 mm) consolidating said layup of wafers under heat and pressure to set adhesive coating said wafers and consolidate said layup into said panel having a substantially uniform density to width profile and cutting the panel along spaced longitudinally extending lines to divide said panel into a plurality of discrete lumber lengths having a width equal to the spacing between said longitudinal cuts.

Preferably the consolidating conditions will be controlled to yield a panel having a substantially uniform density to thickness profile.

Preferably the density of the lumber products so produced will be in the order of 25 lb/ft³ (0.4 g/cm³) through 50 lb/ft³ (0.8 g/cm³). Also preferably the density will not deviate more than 3% from the mean through the panel thickness.

### BRIEF DESCRIPTION OF THE DRAWINGS

Further features, objects and advantages will be evident from the following detailed description of the preferred embodiments the present invention taken in conjunction with the encompanying drawings in which
Figure 1 is a schematic plan view of a plan for carrying out the present invention.

Figure 2 is a schematic side elevation of the plan of Figure 1.

Figure 3 is a partial plan view of a board or panel constructed in accordance with the present invention, illustrating the lay of wafers therein.

Figure 4 is a sectional view along the line 4-4 in Figure 3.

Figure 5 is a graph of density versus thickness illustrating a preferred density profile with thickness through the board of Figure 4.

Figure 6 is a sectional view along the line 6-6 in Figure 4.

### DESCRIPTION OF PREFERRED EMBODIMENTS

The term wafer used throughout this disclosure is intended to define wood particles formed by a waferizer as distinct from pulp chips, sawdust, particles or lengths cut directly from a round log or formed by clipping veneer. The size of the sliced wafers used with the present invention, particularly the length which is always measured in the fiber direction, i.e. parallel to the longitudinal axis of the fibers, is critical to obtaining the required strength to provide a lumber product to replace conventional lumber with a product having essentially the same strength as the lumber being replaced and without a significant change in density.

Referring to Figure 1, adhesive coated wood wafers are brought to the layup forming equipment via a suitable in-feed device wherein the wafers are relatively uniformly laterally spread and are then fed to an orienting device 12 (see for example U.S. Patent 4,494,969 issued January 22, 1985 to Knudson et al) that orients the wafers with their longitudinal dimensions substantially aligned as will be described in more detail here below. In the illustrated arrangement the mat 14 so formed has a substantially uniform density to width profile and is either layed on a caul plate and transported to a press such as a multiopening press schematically illustrated in 16 or is carried by a continuous belt or the like to a continuous press 16 and the mat or layup 14 is pressed and consolidated to form a panel 18, say a panel having a total width of 8 feet (2400 mm) and the required thickness (e.g. for nominal 2 inch (50 mm) lumber the consolidated panel must have a 1-1/2 inch (38 mm) thickness). If a continuous press 16 is used panel 18 is continuously moved from the press 16 in the direction of arrow 20, i.e. in the longitudinal direction of the wafers which is the direction in which the wood fibers are aligned in the wafer, into the cutting station 22. If the press 16 is not a continuous press, i.e. is a multiopening press or the like the mat 14 is carried on a caul plate to be consolidated into a panel, the panel will be withdrawn as indicated by arrow 20, separated from their respective caul plates (not shown) and fed one following the other in the direction of the arrow 20, i.e. with the length of the wafers aligned with the arrow 20 into cutting station 22.

Cutting station 22 as schematically illustrated is made up of a purality of spaced circular saws or cutters 24 axially moveably mounted via hubs 26 on a shaft 28. Hubs 26 are mounted in a conventional manner to be driven by the shaft 28 and yet slidable axially on shaft 28 so that the position of the saws 24 may be adjusted thereby adjust the width of the spaces between the saws which determines the width as indicated by the dimensions W1, W2, W3, etc of the lumber products 30 formed from panel 18 (which may be any appropriate width). Figure 2 further provides a schematic illustration of an automatic spacing device adapted to adjust spacing between saws 24 including a yoke 32 that engages its respective hub 26 and is moved along a shaft 34 by a suitable drive bar 36. There will be one drive bar 36 for each yoke 32 and one yoke 32 for each of the blades 24 to in known manner adjust the position of the saw 24 along the shaft 28. Generally the spacing of the saws or cutters 24, i.e. widths W1, W2, etc, will be greater than the thickness T of the panel.

The two outermost blades, i.e. the top and bottom blade 24 in Figure 1 are used to trim the panel 18 and provide trimmed strips as indicated at 38.

A suitable cut off saw schematically indicated at 40 traverses the panel 18 after the appropriate length of cut boards 30 has passed the saws 24 to cut the boards off to the required lengths. In continuous operation the saw 40 will move both transversely and longitudinally so that a square cut is provided across the width the panel 18 (see the arrows 42 and 44 in Figure 1) and where discrete panels 18 are formed on caul plates the cut off saw may not be necessary but may be useful for trimming to length.

It is intended that press 16 be operated as above indicated to provide a panel 18 of adequate strength which requires that wafers having at least an average length of about 8 inches (200 mm) (length is always considered as measured in direction of the grain of the wafer) preferrably an average length of 10 to 24 inches (250-600 mm) be used. Normally such wafers will be cut at an average thickness not exceeding 0.15 inches (4 mm), preferably less than 0.1 inches (2.5 mm) with the thicker wafers normally being used to produce the thicker panel. The wafers will preferably have an average width of at least 0.25 inches (6 mm), more preferably at least 0.5 inches (12 mm) and in many cases will have a width to thickness ratio of over about 10.

The wafers must be oriented with their length direction aligned relative to the longitudinal direction of the lumber which as above indicated is formed by cutting substantially parallel to the longitudinal direction of the panel 18 or parallel to the direction of outfeed from the press 16. This orientation will never be 100% in the machine direction, i.e. parallel to the longitudinal axis of the panel 18 and the axial length of the lumber products 30, but will be such that the mean deviation of the wafer lengths (fiber direction) from the longitudinal axis of the panel 18 and thus form the longitudinal axis of the lumber product is within the range of approximately 0 to 10 degrees when measured in the major plane of the panel 18, i.e. measured on say the upper surface of the panel 18 as indicated at 46 in Figures 2 and 3. The mean deviation measured in a plane extending longitudinally to the panel 18 or boards 30 say parallel to the cut faces formed by the saws 24 (i.e. perpendicular to the plane 46) will normally be in the range of 0 to 5 degrees as schematically illustrated by the angle A in Figure 4. The angle A will preferably be small closer to the 0 to 3 degrees since if the angle A is too large and wafers extend almost from one major surface of the panel to the other, a weak product will be produced and this must be avoided.

Press cycle will be controlled (including the rate of change of temperature assuming a continuous press) depending on the product to be produced but normally will be such that the density to thickness profile is substantially constant, i.e. a deviation of less than 3% from the mean for a normal lumber product. Generally the faces of the panel 18 contacting the press plates will have a slightly higher density than the central portion of the panels. If the lumber product is to be used as planking, i.e. with the loading perpendicular to the major face, it may be desirable to manufacture a panel with distinct core and surface layers with the surface layers having a significantly higher density than in the core. With a plank the deviation in density from the mean may be as high as 10% depending on the relative thickness of the dense surface layers to the less dense core portion.

The uniform profile of density to thickness is significantly more important with the structural lumber product of the present invention which will normally be loaded perpendicular to its cut or edge face, i.e. parallel to the face represented by surface 46 of panel 18 so that the major faces of the panel which contact the platens of the press will be aligned with the load and the center or core of the panel no longer forms the neutral axis when the structural member is being stressed.

In the operation of the present invention suitable wafers as above described are first formed in a mat 14 of approximately 4 times the desired finished thickness of the panel 18 which will normally limit the maximum thickness of the panel to about 4 inches (100 mm). The wafers will be precoated with adhesive normally a phenol formaldehyde resin although isocyanates may also be used or any other suitable adhesive. Normally if phenol formaldehyde is used a dried powdered resin will be used although with proper application a wet or liquid resin may also be used. Change in resin may require a change in the pressing schedule to ensure proper curing of the resin when the mat is under pressure.

Assuming the lumber to be produced is nominal 2 inch (50 mm) thick lumber then the thickness of the panel 18 will be 1-1/2 inch (40 mm) and the cutters 24 will be separated to cut the panel 18 into strips and to produce a 2 × 6; 2 × 8; 2 × 10; 2 × 12; or even 2 × 16 inch; etc, lumber as desired. Generally the wider the width dimension the more valuable the product yet it is as easy to manufacture a 2 × 16 inch board as it is to manufacture a 2 × 4 utilizing the present invention and any desired product mix may be made. Furthermore, if a continuous press is used the length of the boards so formed is determined simply by activation of the cutoff saw 40 to cut the boards to the desired length. If caul plates are used the saw 40 may simply be used to trim the lumber to length or alternatively it could be trimmed at some other stage. In this case the maximum length is determined by the length of the caul plate.

### EXAMPLE 1

A single layer oriented wafer mat was hand felted aspen wafers onto an 8 foot (2400 mm) long caul plate. The wafers used were 12 inches long and 0.025 inches (0.6 mm) thick and 1-1/4 inch (30 mm) wide and were produced at MacMillan Bloedel's Thunder Bay Division. 5% powder phenol formaldehyde resin and 2% slack wax were applied to the wafers. A matching 8 foot caul plate was placed on top of the mat before pressing. The felted wafer mat was then advanced through a hot press (in the Research Centre under lab conditions) in 2 foot stages. Each stage was pressed for 20 minutes at a press temperature of 210°C. The resulting product had a thickness of 1-1/2 inches and an average density of 40 lb/ft³ (0.64 grams/cc). The modulus of elasticity (MOE) of the section so produced was 1,697,000 psi (11.70 GPa) measured while applying forces parallel to the faces formed by the caul plates, i.e. in a direction equivalent to perpendicular to the cut faces of the lumber product.

It will be apparent that the pressing of this sample was not under ideal conditions so that the panel produced was far from ideal. However the sample clearly indicates that the modulus of elasticity (MOE) is at least equivalent to that for conventional lumber of the grade specified and at a reasonable density.

### EXAMPLE 2

In a further attempt to determine the applicability of utilizing wafers that are relatively inexpensive, a relatively thin aspen veneer 0.05 inch (1 mm) thick at 10% moisture content was clipped to 12 inch length by 1/2 inch width strips to make an 8 foot long, 11 inch wide by 2-1/2 inch thick oriented lumber billet utilizing a continuous press, microwave heating, 6% powdered phenol formaldehyde resin and 2% slack wax. A mat was formed from wafers precoated with adhesive and oriented to substantially align with the length of the lumber product and passed through the press over a period of 9 minutes. The average density of the resultant lumber was 40 lb/ft³ (0.64 grams/cc) at 12% moisture and the resulting board had an average MOE of 1,650,000 psi add a modulus of rupture (MOR) of 6900 psi.

Another board made in a similar manner had a density of 33.75 lb/ft³ (0.54 g/cc), a MOE of 1,500,000 psi and a MOR of 5,500 psi.

Examples 1 and 2 clearly demonstrate that it is practical to manufacture lumber products having acceptable physical characteristics for structural lumber applications when made from a species such as aspen which is not a good species for such materials and at a final density that while higher than aspen is similar to that of many species.

Having described the invention modifications will be evident to those skilled in the art without departing from the spirit of the invention as defined in the appended claims.

## Claims

1. A lumber product having a thickness of at least 1 inch (25 mm) which has been cut from a panel made of elongate wood particles oriented with their lengths having a mean deviation of 0-10° from the longitudinal axis of the panel measured in a major plane of the panel and a mean deviation of 0-5° measured in a minor plane extending longitudinally of the panel and perpendicular to the major plane, the lumber product having a pair of cut edges spaced to define its width and extending substantially parallel to the longitudinal axis of the panel from which the lumber is cut, characterised in that the wood particles are wafers formed by a waferizer and having a thickness of less than 2.5 mm (0.1 inch), a width of at least 12 mm (0.5 inch), a width-to-thickness ratio of over 10 and an average length measured in the grain direction of at least 8 inches (200 mm), whereby the lumber product is suitable for use as a structural lumber product having a Modulus of Elasticity of at least 10.34 GPa (1,500,000 psi) at a density equivalent to 643.2 Kg/m³ (40 lbs. per cubic foot).

2. A lumber product according to claim 1, characterised in that it has a density within the range of 25-50lb/ft³ (0.4-0.8 g/cm³).

3. A lumber product according to claim 1 or claim 2, characterised in that the wafers have a thickness which is less than 0.05 inch (1.25 mm).

4. A lumber product according to any one of claims 1-3, characterised in that the wafers have a mean length of between 10 and 24 inches (250 and 600 mm).

5. A lumber product according to any one of claims 1-4, characterised in that it has a substantially uniform density to thickness profile.

6. A lumber product according to any one of claims 1-4, characterised in that it has a density profile to thickness with a deviation from the mean density of less than 3%.

7. A method of making lumber products from a mat of elongate wood particles which are oriented in the mat with their lengths having a mean deviation of 0-10° from the longitudinal axis of the mat measured in a major plane thereof and a mean deviation of 0-5° measured in a minor plane extending longitudinally of the mat and perpendiculr to the major plane, characterised by:
(a) producing the wood particles as wafers in a waferizer, the wafers having an average length measured in the grain direction of at least 200 mm (8 inches), a thickness of less than 0.25 mm, a width of at least 12 mm and a width to thickness ratio of over 10 i
(b) consolidating the mat under heat and pressure to bind the wafers together using an adhesive pre-applied to the wafers and thus forming a panel; and
(c) cutting the panel longitudinally at spaced-apart locations to divide the panel into a plurality of lumber products each having a width determined by the spacing of the cuts and a thickness determined by the thickness of the panel, the longitudinal cuts being aligned with the longitudinal axis of the mat.

8. A method according to claim 7, characterised in that consolidating the mat to form the panel is under conditions to produce a panel having a substantially uniform density profile with thickness of the panel.

## Patentansprüche

1. Holzprodukt mit einer Stärke von zumindest 1 Zoll (25 mm), welches geschnitten ist aus einer Tafel aus langgestreckten Holzteilchen, die mit ihren Längserstreckungen derart ausgerichtet sind, daß ihre mittlere Abweichung von der Längsachse der Tafel, gemessen in einer Hauptebene der Tafel, zwischen 0 bis 10° liegt, und eine Abweichung von 0 bis 5°, gemessen in einer Nebenebene, die sich längs der Tafel und senkrecht zu der Hauptebene erstreckt, gegeben ist, wobei das Holzprodukt ein Paar von Schneidkanten aufweist, die beabstandet sind und die Breite des Produktes bestimmen und sich im wesentlichen parallel zur Längsachse der Tafel erstrecken, von der das Holzprodukt geschnitten ist, dadurch gekennzeichnet, daß die Holzteilchen Plättchen sind, die durch einen Scheibenbildner geformt sind und eine Dicke von weniger als 2,5 mm (0,1 inch), eine Breite von zumindest 12 mm (0,5 inch), ein Breite-zu-Dicke-Verhältnis von mehr als 10 und eine mittlere Länge, gemessen in Faserrichtung, von zumindest 8 Zoll (200 mm) aufweisen, wodurch das Holzprodukt geeignet ist zur Verwendung als tragendes Holzprodukt mit einem Elastizitätsmodul von zumindest 10,34 GPa (1,500,000 psi) bei einer Dichte, die 643,2 kg/m³ entspricht (40 lbs. pro Kubikfuß).

2. Holzprodukt gemäß Anspruch 1, dadurch gekennzeichnet, daß es eine Dichte im Bereich von 25 bis 50 lb/ft³ (0,4 bis 0,8 g/cm³) aufweist.

3. Holzprodukt gemäß einem der Ansprüche 1 oder 2, dadurch gekennzeichnet, daß die Scheibchen eine Dicke aufweisen, die geringer ist als 0,05 Zoll (1,25 mm).

4. Holzprodukt gemäß einem der Ansprüche 1 bis 3, dadurch gekennzeichnet, daß die Scheibchen eine mittlere Länge aufweisen, die zwischen 10 und 24 Zoll (250 und 600 mm) liegt.

5. Holzprodukt gemäß einem der Ansprüche 1 bis 4, dadurch gegekennzeichnet, daß es im wesentlichen ein gleichförmiges Dichte-zu-Stärke-Profil aufweist.

6. Holzprodukt gemäß einem der Ansprüche 1 bis 4, dadurch gekennzeichnet, daß es ein Dichte-zu-Stärke-Profil aufweist mit einer Abweichung von der mittleren Dichte von zumindest 3 %.

7. Verfahren zum Herstellen von Holzprodukten aus einer Matte aus langgestreckten Holzteilchen, die in der Matte derart orientiert sind, daß ihre Längen eine mittlere Abweichung von 0 bis 10° in bezug auf die Längsachse der Matte, gemessen in einer Hauptebene derselben, aufweisen, und eine mittlere Abweichung von 0 bis 5°, gemessen in einer Nebenebene, die sich längs der Achse und senkrecht zu ihrer Hauptebene erstreckt, gekennzeichnet durch:
(a) Erzeugen von Holzteilchen als Plättchen in einem Scheibchenbildner, wobei die Plättchen eine mittlere Länge, gemessen in der Faserrichtung, von zumindest 200 mm (8 Zoll) aufweisen, sowie eine Dicke von weniger als 0,25 mm, eine Breite von zumindest 12 mm und ein Verhältnis der Breite zur Dicke von mehr als 10,
(b) Verfestigen der Hatte unter Hitze- und Druckeinwirkung, um die Plättchen aneinander zu binden unter Verwendung von Klebstoff, der zuvor auf die Plättchen aufgebracht wurde, und Bilden einer Tafel hierdurch; und
(c) Schneiden der Tafel in Längsrichtung an voneinander beabstandeten Orten, um die Tafel in eine Mehrzahl von Holzprodukten zu unterteilen, von denen jedes eine Breite aufweist, die bestimmt ist durch den Abstand der Schneidflächen, und eine Stärke, die bestimmt ist durch die Stärke der Tafel, wobei die Längsschnitte ausgerichtet sind in Richtung auf die Längsachse der Matte.

8. Verfahren nach Anspruch 7, dadurch gekennzeichnet, daß die Verfestigung der Matte zur Bildung einer Tafel unter solchen Bedingungen erfolgt, daß eine Tafel erzeugt wird, die im wesentlichen eine gleichförmige Dichte als Funktion des Abstandes von der Oberfläche der Tafel aufweist.

## Revendications

1. Produit du type bois d'oeuvre présentant une épaisseur d'au moins 25 mm (1 pouce), qui a été découpé à partir d'un panneau fait de particules de bois de forme allongée, orientées avec leur longueur présentant une déviation moyenne de 0-10° par rapport à l'axe longitudinal du panneau, mesurée dans un plan principal du panneau et une déviation moyenne de 0-5°, mesurée dans un plan secondaire s'étendant selon la direction longitudinale du panneau et perpendiculairement au plan principal, le produit du type bois d'oeuvre présentant une paire de bords coupés, espacés l'un de l'autre pour définir sa largeur, et s'étendant sensiblement parallèlement à l'axe longitudinal du panneau à partir duquel le bois d'oeuvre est coupé, produit caractérisé par le fait que les particules de bois sont des tranches formées par une trancheuse et présentant une épaisseur de moins de 2,5 mm (0,1 pouce), une largeur d'au moins 12 mm (0,5 pouce), un rapport largeur-épaisseur supérieur à 10 et une longueur moyenne, mesurée selon le fil, d'au moins 200 mm (8 pouces), ce par quoi le produit du type bois d'oeuvre convient pour emploi comme produit du type bois d'oeuvre de structure présentant un module d'élasticité d'au moins 10,34 GPa (1 500 000 psi) avec une densité équivalente à 643,2 kg/m³ (40 livres par pied cubique).

2. Produit du type bois d'oeuvre selon la revendication 1, caractérisé par le fait qu'il présente une densité sur la plage de 0,4 - 0,8 g/cm³ (25-50 livre/pied cube)

3. Produit du type bois d'oeuvre selon la revendication 1 ou la revendication 2, caractérisé par le fait que les tranches ont une épaisseur qui est inférieure à 1,25 mm (0,05 pouce).

4. Produit du type bois d'oeuvre selon l'une quelconque des revendications 1-3, caractérisé par le fait que les tranches ont une longueur moyenne valant entre 250 et 600 mm (10 et 24 pouces).

5. Produit du type bois d'oeuvre selon l'une quelconque des revendications 1-4, caractérisé par le fait qu'il a une densité sensiblement uniforme sur toute l'épaisseur.

6. Produit du type bois d'oeuvre selon l'une quelconque des revendications 1-4, caractérisé par le fait que, sur toute l'épaisseur, sa densité s'écarte de moins de 3% de la densité moyenne.

7. Procédé de fabrication de produits du type bois d'oeuvre à partir d'un tapis de particules de bois de forme allongée qui sont orientées dans le tapis avec leur longueur présentant une déviation moyenne de 0-10° par rapport à l'axe longitudinal du tapis, mesurée dans son plan principal, et une déviation moyenne de 0-5°, mesurée dans un plan secondaire s'étendant selon la direction longitudinale du tapis et perpendiculairement au plan principal, procédé caractérisé par les étapes suivantes:
(a) produire les particules de bois sous forme de tranches dans une trancheuse, les tranches présentant une longueur moyenne, mesurée selon le fil, d'au moins 200 mm (8 pouces), une épaisseur de moins de 0,25 mm, une largeur d'au moins 12 mm et un rapport largeur-épaisseur supérieur à 10,
(b) consolider le tapis par la chaleur et sous pression pour lier ensemble les tranches en utilisant un adhésif pré-appliqué aux tranches, formant ainsi un panneau; et
(c) couper le panneau dans le sens longitudinal en des positions espacées l'une de l'autre, pour diviser le panneau en une pluralité de produits du type bois d'oeuvre, présentant chacun une largeur déterminée par l'espacement des coupes et une épaisseur déterminée par l'épaisseur du panneau, les coupes longitudinales étant alignées avec l'axe longitudinal du tapis.

8. Procédé selon la revendication 7, caractérisé par le fait que la consolidation du tapis pour former le panneau se fait dans des conditions permettant de produire un panneau présentant une densité sensiblement uniforme sur toute l'épaisseur du panneau.
